

May 26, 1959

E. F. EVANS

2,888,317

PRODUCTION OF POLYACRYLONITRILE FILAMENTS  
OF HIGH UNIFORM DENSITY

Filed April 10, 1953

2-Sheets-Sheet 1

FIG. 1.



INVENTOR

Evan F. Evans

BY *C. H. Mortenson*

ATTORNEY

May 26, 1959

E. F. EVANS

2,888,317

PRODUCTION OF POLYACRYLONITRILE FILAMENTS  
OF HIGH UNIFORM DENSITY

Filed April 10, 1953

2 Sheets-Sheet 2

FIG. 2.



FIG. 3.



INVENTOR

Evan F. Evans

BY

*C. Dr. Mortenson*

ATTORNEY

1

2,888,317

## PRODUCTION OF POLYACRYLONITRILE FILAMENTS OF HIGH UNIFORM DENSITY

Eyan F. Evans, West Chester, Pa., assignor to E. I. du Pont de Nemours and Company, Wilmington, Del., a corporation of Delaware

Application April 10, 1953, Serial No. 347,986

13 Claims. (Cl. 18—54)

This invention relates to improved shaped articles, such as fibers, filaments, yarns and similar items and to a process for producing them. More specifically, the invention is directed to producing fiber structures of acrylonitrile homopolymers and of acrylonitrile copolymers wherein the acrylonitrile content is at least 85%, which structures are more uniform than those produced heretofore, especially with respect to dyeability.

One method of manufacturing polyacrylonitrile yarns is by dry or evaporative spinning of polymer solutions. The yarn collected from the spinning cell may contain upwards of 10% solvent and frequently at least 30% solvent. The recovery of the solvent is essential for economic operation, but the recovery of this residual solvent is complicated by the fact that the "as spun" yarn must undergo further processing to provide it with desirable textile properties.

The most important of these steps is drawing or stretching to several times its "as spun" length, i.e. from 2 to 10 times or more. The condition of the yarn as it is subjected to this stretch is all important if optimum properties are to be attained in the drawn product. One of the essential requirements for uniformity of results is a low and uniform solvent content of the yarn entering the steam stretching chamber. The removal of solvent from the spun yarn can be accomplished by water or aqueous liquor washing and this has been done very successfully by pressure washing wound packages of the yarn.

The removal of solvent from the yarn by washing with cold water, however, produces a porous structure of low density. It was found that this excessive porosity, which is undesirable, could be largely avoided by washing with water or water containing a minor amount of solvent heated to an elevated temperature such as 100° C. This high temperature washing was considered desirable until it was found that drawing of this yarn could not be accomplished without having short length non-uniformities in dyeing. Subsequently, it was found that while the average density of the drawn yarn of acrylonitrile homopolymer was relatively high, being about 1.17, there were short lengths which were less dense, such as 1.14. This difference very markedly affected dyeing uniformity for the low density sections dyed much deeper, imparting short length deep-dyeing flashes to the fabric made thereof.

It is, therefore, an object of this invention to provide a novel process for the production of yarns, filaments, fibers and like structures of acrylonitrile homopolymers or of copolymers wherein the acrylonitrile content is at least 85%, which structures are characterized by more uniform dyeability. Other objects of this invention will be apparent from the description that follows.

The objects of this invention are accomplished by spinning a solution of an acrylonitrile homopolymer or of a copolymer wherein the acrylonitrile content is at least 85% to produce a filamentary structure having, at the point of collection, at least about 5% solvent, washing

2

the structure with an aqueous liquid at a temperature below about 50° C. until the solvent content of the structure is no more than about 2.5% by weight (based on the dry weight of the structure), drying the structure at a temperature below about 110° C. to produce a substantially undrawn structure containing no more than 7% by weight of water and thereafter drawing 2 to 10 times or more. The stretching or orientation step is usually accomplished at an elevated temperature, for example, at 100° C. or above. Preferably, the water content is between about 2% and about 4% by weight.

Figure I shows the effect of the temperature used in the extraction on the density of undrawn yarn air dried at 25° C.;

Figure II shows the effect of the drying temperature on the density of undrawn yarn which has been solvent extracted at a temperature below 40° C.; and

Figure III shows the effect of the time of extraction on the density of air dried yarn.

20 Washing of the filamentary structures may be accomplished with water or with a dilute aqueous solution of a solvent, usually that used in the spinning solution. Whatever the mode of extraction, the solvent should be removed at least to the extent that no more than about 25 2.5% by weight (based on the dry weight of the structure) is left. Preferably, this solvent content should be reduced below 2.0% and it may be reduced to as little as 1.0% or less with good results. The filamentary structure subjected to washing may be in the form of a wound 30 yarn package on a perforated core in which case pressure washing may be used. It may be washed on the run by leading it through one or more troughs containing the washing liquor or under showers of washing liquor. In the form of skeins or in other readily accessible forms 35 the structures may be subjected to solvent extraction by leaching, dunking or similar methods. Other washing methods or combinations of methods may also be used. It is important that the temperature of the wash liquor be maintained below about 50° C. The wash liquor 40 temperature may be substantially below this level and even below room temperature, i.e. at 5° C. or less; although there is no advantage in cooling the wash liquor below room temperature. Generally, temperatures in the range of from room temperature to about 40° C. will be 45 found most satisfactory.

Drying may be carried out in a number of ways. Warm air drying is very satisfactory as is hot roll drying, provided the air or roll temperature is not allowed to exceed about 110° C. While excellent results have been 50 obtained by air drying at room temperature, drying at temperatures above about 70° C. is preferred. It is important to dry down to below about 7% moisture content of the yarn and preferably to about 2% to 4% moisture. With increasing amounts of moisture above 7%, the resultant yarns dye less and less uniformly.

It is indeed surprising that the combination of critical 55 low temperature solvent extraction with critical drying produces a high density structure which is very much improved in uniformity of density since low temperature solvent extraction without drying results in a drawn 60 yarn of very low density, i.e. of the order of 1.11 or less. While high temperature (100° C.) solvent extraction followed by high temperature (105° C.) drying gives high density yarn structures, the density uniformity is not

65 nearly as good as when low temperature solvent extraction with drying is practiced. High temperature (100° C.) solvent extraction followed by low temperature (25° C.) drying gives unusually low density structures before drawing and still greater density non-uniformity. Table 70 I below shows comparative figures on densities of yarns after extraction and drying in accordance with the invention but before drawing and the "standard deviation"

for each of the different conditions shown. Density uniformity is at least about 2 times better when low temperature extraction with drying is used.

TABLE I

| Extraction Temp., °C. | Drying Temp., °C. | No. of Samples | Average Density | Standard Deviation |
|-----------------------|-------------------|----------------|-----------------|--------------------|
| 25                    | 25-30             | 23             | 1.173           | 0.0051             |
| 25                    | 105               | 23             | 1.180           | 0.0043             |
| 100                   | 25                | 22             | 1.133           | 0.012              |
| 100                   | 105               | 22             | 1.173           | 0.010              |

To compare density values of some drawn yarns under different conditions of processing, Table II below is given. It will be noted here too that there are some changes in density in undrawn versus drawn yarn.

TABLE II

| Extraction Temp., °C. | Drying Temp., °C. | Density        |               |
|-----------------------|-------------------|----------------|---------------|
|                       |                   | Before Drawing | 8X Drawn Yarn |
| 25                    | 25                | 1.172          | 1.177         |
| 25                    | 105               | 1.182          | 1.180         |
| 25                    | undried           | -----          | <1.111        |
| 100                   | 25                | 1.137          | 1.184         |
| 100                   | undried           | -----          | 1.175         |

From the curves plotted in Figure I it is noted that high density filaments result from "as spun" yarns extracted at temperatures below about 50° C. and dried at 25° C. Above 50° C., the densities fall off and become variable whereas at about 50° C. or below, the densities are constant and high. Furthermore, whether the yarn is completely relaxed (curve A) or restrained (curve B) from relaxation during extraction makes little or no difference at these lower temperatures of extraction. Higher temperatures of drying do yield a yarn of the greater density as is shown in Figure II. In this figure density curves again are plotted, this time on data resulting from low temperature (below 40° C.) aqueous extraction of solvent from the "as spun" yarn after which the washed yarn is dried at temperatures ranging from 40° C. to 135° C. One set of data plotted is on yarn dried under just sufficient tension to maintain its wet length (curve C) while the other set of data is on yarn dried without any tension (curve D). Here it will be noted the curves coincide in temperatures above 80° C. and variations in tension as may develop in drying yarn will not cause substantial differences in density when the yarns are dried at temperatures above about 70° C. For this reason, temperatures between 70° and 110° C. are preferred.

Another set of data showing the desirability of low temperature extraction over higher temperatures of extraction for a period of time ranging from one second up to several hours is shown by the curves in Figure III. Herein it is noted that the time of extraction at 25° C. has no effect on the density of the yarn, whereas at 60°, 75° and 100° C., the time of extraction importantly affects the density of the yarn. Thus, by conducting solvent extraction at a low temperature and following this step by drying, preferably at a temperature between 70° and 110° C., the density of the resulting yarn before and after drawing will be relatively high and more uniform than obtainable under other operating conditions. While uniform density yarn per se may not result in uniform dyeing yarn, it appears from the data collected that uniform dyeing yarn cannot be secured without uniformity of yarn density.

In the examples that follow additional illustrations of

preferred methods of applying this invention are given. These examples are given for illustrative purposes only.

#### Example I

5 A 640 denier-40 filament yarn produced by evaporative spinning of an acrylonitrile homopolymer from solution in N,N-dimethylformamide was wound up at the spinning machine on a perforated core. This yarn contained about 40% solvent (based on the dry solvent-free weight of the yarn) and was subjected to solvent extraction by pressure washing with water at room temperature. The washed yarn was skeined and dried at room temperature on swifts which allowed the yarn to shrink upon drying. The dried yarn was subjected to steam drawing to eight times its dry undrawn length followed by 9.5% hot relaxation. A piece of tubing knitted from this yarn and dyed with a Celanthrene Pure Blue BRS was free of dyeing non-uniformities.

#### Example II

20 475 denier-30 filament acrylonitrile homopolymer yarn dry spun from solution in N,N-dimethylformamide and collected on perforated cores while it contained about 35% solvent (based on the dry and solvent-free weight of the yarn) was pressure washed with water containing 2% N,N-dimethylformamide for 2 hours, at the end of which time the solvent content of the yarn had been reduced to about 2% (based on the dry weight of the yarn). The yarn was subjected to drying by means of 25 heated rolls, varying the roll contact and the temperature of the rolls to produce samples having different moisture contents as they were subjected to pressure steam drawing. The steam pressure was varied to give good drawing to eight times the undrawn length and the resulting drawing tensions are recorded with the other data in Table III below. After drawing, the yarn was heat relaxed 30 12%.

TABLE III

| 40 | Sample | Drying Roll Temp., °C. | Roll Contacts | Percent Moisture Content of Dried Yarn | Dyeing Uniformity | Draw Tension, Grams | Steam Pressure For Drawing, Pounds/Sq. In. |
|----|--------|------------------------|---------------|----------------------------------------|-------------------|---------------------|--------------------------------------------|
| 45 | 1----- | 85                     | 12            | 3.8                                    | good-----         | 30                  | 55                                         |
|    | 2----- | 85                     | 21            | 2.9                                    | excellent-----    | 30                  | 44                                         |
|    | 3----- | 85                     | 21            | -----                                  | do-----           | 40                  | 30                                         |
|    | 4----- | 80                     | 30            | 2.4                                    | do-----           | 30                  | 32                                         |
|    | 5----- | 80                     | 30            | -----                                  | do-----           | 50                  | -----                                      |
| 50 | 6----- | 110                    | 9             | 2.3                                    | good-----         | 32                  | 54                                         |

It will be noted that all samples dried to below 3% moisture at 80° to 85° C. showed excellent dyeing uniformity, the dye test being on knitted tubing dyed with Celanthrene Pure Blue BRS.

#### Example III

Acrylonitrile homopolymer yarn dry spun from solution in N,N-dimethylformamide and collected on a perforated core as 510 denier-30 filament yarn containing about 35% solvent (based on the dry and solvent-free weight of the yarn) was pressure washed with water at a temperature of 40° C. for 3½ hours at which time the solvent was reduced to about 1.8% (based on the dry and solvent-free weight of the yarn). This yarn was then 60 dried on the run by passing it twelve times around the contact drying roll heated to 97° C. to reduce the moisture content of the yarn to about 2.9%. It was drawn eight times in a steam drawing chamber and thereafter the yarn was heat relaxed 10%. The drawn yarn had 65 a density of 1.179 and comparable physical properties to yarn prepared by hot water washing and drawing without drying. The yarn produced from this test, when knitted into tubing and dyed with Celanthrene Pure Blue BRS, showed excellent dyeing uniformity. It was free 70 of short length deep dyeing flashes and showed no dye

junctions where the yarn from the outside of the spinning package joined yarn from the inside of the same or different spinning package. A control yarn was similarly produced, except that it was washed at a temperature of 105° C. and was drawn without drying; in dyeing tests there were a number of short length deep dyeing flashes, especially in yarn from the outside of the spinning cake and a distinct dye junction between "inside" and "outside" yarn, the inside yarn being lighter. Also, yarn was subjected to the same step of solvent extraction but dried before drawing by contact with rolls heated to 130° C.; this reduced the moisture content of the yarn to below 2% and non-uniform dyeing yarn similar to the "control" yarn resulted.

*Example IV*

A copolymer of acrylonitrile and methylacrylate 94/6 was dry spun from solution in N,N-dimethylformamide and wound up as 510 denier-30 filament yarn containing about 30% residual solvent. The yarn was trough extracted in countercurrent flowing water at 30° C. and then dried at room temperature. The dried undrawn yarn had a density of 1.181. It was pressure steam drawn eight times and then hot relaxed 12% to give a deep and uniform dyeing yarn free of short length variability.

*Example V*

An acrylonitrile homopolymer dry spun yarn which was subjected to continuous trough extraction in countercurrent flowing water at 25° C. followed by 90° to 110° C. roll drying and thereafter steam drawn and relaxed showed good dyeing uniformity, whereas yarns similarly trough extracted with water at temperatures of 25° C. and 95° C. and steam drawn without previously drying exhibited very non-uniform dyeing. Also, yarns trough extracted at 95° C. followed by 90° or 110° C. roll drying before steam drawing exhibited non-uniform dyeing.

*Example VI*

Acrylonitrile homopolymer dry spun yarns were collected at the spinning machine on perforated cores in the form of square ended packages with the aid of self-traversing rolls. These packages were effectively pressure washed with water or aqueous liquor containing up to 3% solvent (N,N-dimethylformamide) at temperatures of from 20° C. to 40° C. and thereafter dried on 95° C. rolls before steam drawing and hot relaxing. This yarn drawn eight times exhibited good dyeing uniformity, whereas yarn similarly extracted but dried on 125° C. rolls displayed numerous non-uniformities in dyed knitted tubing.

In other tests it has been shown that solvent extraction from dry spun acrylonitrile homopolymer yarn at 30° C. followed by drying at the same temperature, the yarn being free to shrink during both treatments, resulted in isotropic shrinkage of the yarn, this shrinkage being the result of the decrease in yarn volume due to its solvent loss. In contrast, hot extraction followed by drying, hot or cold, resulted in greater longitudinal shrinkage than the isotropic value. It follows then that by the practice of this invention, yarns of more uniform denier can be obtained as well as improved uniformity in dyeing.

Copolymer yarns wherein the acrylonitrile content is at least 85% behave in general much the same as the homopolymers. For instance, water extraction for one hour of acrylonitrile/methylacrylate 94/6 copolymer yarn dry spun from solution in N,N-dimethylformamide showed a maximum air dried density of 1.181 when extraction was at 29° to 48° C., while extraction at temperatures above 60° C. gave lower and variable air dried density. At 60° C. extraction, the density was 1.143; at 70° C., 1.137; at 79° C., 1.121 and at 90° C., 1.137.

However, in some instances an acrylonitrile copolymer yarn is more detrimentally affected by high temperature extraction than is the homopolymer yarn. For example, an acrylonitrile/methylacrylate 94/6 copolymer yarn

was found to develop numerous cracks within the yarn core or show separation of the yarn skin from the yarn core (shown by microscopic dyed cross-sections), depending on spinning and packaging history. On the other hand, low temperature extraction with an attendant slower extraction rate, did not develop any skin/core interdependence such as was found to result from hot extraction. The process of this invention avoids the possibility of this cracking effect.

10 The improvement in density and dyeing uniformity which follows from the practice of this invention are the outstanding benefits realized and these improvements are indeed important if not essential for the continued commercial acceptance of the yarn. Short length dyeing

15 flashes have been present in more or less pronounced form and to a greater or lesser extent since the beginning of manufacture of acrylonitrile polymer yarns. As earlier stated, a change in density from 1.17 to 1.14 causes a very decided change in dyeing depth and even 20 a density change of as little as 0.01 is sufficient to bring about a change in depth of color. This invention enables the production of much more uniform density yarn than has been produced heretofore, in many cases with maximum density variation within a single yarn package no 25 greater than about 0.005, and as a result discernible dye differences are substantially eliminated. The process of this invention can be applied effectively to the many acrylonitrile polymers and copolymers disclosed in such patents as U.S. 2,404,714 to 2,404,727. These contain a 30 major amount of acrylonitrile and those of most interest are those that are derived from about 85% or more, by weight, of acrylonitrile.

Generally, packages having unsupported side walls are made. High temperature extraction of these results in 35 package instability and deformation, but by the process of this invention these adverse elements are avoided. In addition to this, differences between inside and outside densities are decreased and dyeing uniformity is attained.

Any modification which conforms to the principles of 40 the invention described herein is intended to be included within the scope of the claims below.

I claim:

1. A process for the production of a filament of high uniform density composed of at least 85% of acrylonitrile which comprises producing by dry spinning a substantially undrawn filament containing at least about 5% of a solvent, based on the dry weight of said filament, by extrusion of a solution of said polymer in said solvent; washing said filament with an aqueous liquid at a 45 temperature below about 50° C. until the solvent content is below about 2.5%, based on the dry weight of said filament; and drying the resultant, extracted filament at a temperature from about 70° C. to about 110° C. to produce a substantially undrawn filament containing no 50 more than about 7% of water, based on the dry weight of said filament.

2. A process in accordance with claim 1 wherein said water content is reduced to about 2% to about 4% based on the dry weight of said filament.

3. A process in accordance with claim 1 wherein said washing produces an extracted filament having less than 2% residual solvent.

4. A process in accordance with claim 1 wherein the temperature of the said aqueous liquid is in the range of about 5° C. to about 40° C.

5. A process in accordance with claim 1 wherein said polymer is polyacrylonitrile.

6. A process in accordance with claim 1 wherein said polymer is a copolymer.

7. A process for the production of a filament of high uniform density composed of at least 85% of acrylonitrile which comprises producing by dry spinning a substantially undrawn filament containing at least about 5% of a solvent, based on the dry weight of said filament, by extrusion of a solution of said polymer in said solvent;

washing said filament with an aqueous liquid at a temperature below about 50° C. until the solvent content is below about 2.5%, based on the dry weight of said filament; drying the resultant, extracted filament at a temperature from about 70° C. to about 110° C. to produce a substantially undrawn filament containing no more than about 7% of water, based on the dry weight of said filament; and stretching the resultant extracted, dried filament to produce an oriented filament.

8. A process in accordance with claim 7 wherein said polymer is polyacrylonitrile. 10

9. A process in accordance with claim 7 wherein said polymer is a copolymer.

10. A process in accordance with claim 7 wherein said resultant extracted, dried filament is stretched at least 15 twice its original length.

11. A process in accordance with claim 7 wherein said water content is reduced to about 2% to about 4% based on the dry weight of said filament.

12. A process in accordance with claim 7 wherein the said resultant, extracted filament has less than 2% residual solvent.

13. A process in accordance with claim 7 wherein the temperature of the said aqueous liquid is in the range of about 5° C. to about 40° C.

References Cited in the file of this patent

UNITED STATES PATENTS

|           |                 |       |                |
|-----------|-----------------|-------|----------------|
| 2,420,565 | Rugeley         | ----- | May 13, 1947   |
| 2,611,929 | Hoxie           | ----- | Sept. 30, 1952 |
| 2,733,121 | Griffith et al. | ----- | Jan. 31, 1956  |
| 2,761,754 | Jones et al.    | ----- | Sept. 4, 1956  |